

Patented July 21, 1925.

1,547,138

# UNITED STATES PATENT OFFICE.

JOHN R. MACMILLAN, OF LA SALLE, NEW YORK, ASSIGNOR TO NIAGARA ALKALI COMPANY, OF NIAGARA FALLS, NEW YORK, A CORPORATION OF NEW YORK.

## BLEACHING PROCESS.

No Drawing.

Application filed September 6, 1924. Serial No. 736,282.

To all whom it may concern:

Be it known that I, JOHN R. MACMILLAN, a citizen of the United States, residing at La Salle, in the county of Niagara and 5 State of New York, have invented certain new and useful Improvements in Bleaching Processes, of which the following is a specification.

This invention relates to bleaching processes; and it relates to a method of bleaching fiber wherein such fiber is treated with a modicum of bleaching solution (hypochlorite) and with chlorin and finally with enough more bleaching solution to accomplish the degree of bleaching desired; such 15 process being particularly applicable to ligniferous fibers rich in lignin, such as jute, but also applicable to other fibers; all as more fully hereinafter set forth and as 20 claimed.

In bleaching all sorts of fibers and fabrics it has of course long been the practice to treat the fiber with a bleaching liquor containing a hypochlorite; this bleaching liquor 25 containing hypochlorite of calcium, of sodium, or of potassium as the case may be. A solution of bleaching powder (which contains calcium hypochlorite) is often used. Sometimes bleaching liquor is made by chlorinating a caustic soda solution. Afterwards 30 the fabric is washed, etc., and is, in some cases, treated with an antichlor. This method of bleaching has been known and used for many years. For some purposes, as in 35 bleaching paper pulp, it has been found more convenient to use a preliminary treatment with chlorin before treating with the regular bleaching liquor. Part of the bleaching is done by the chlorin and the rest 40 by the bleaching liquor.

With many fibers there is a practical limit to the extent to which bleaching can be carried in these ways, this being particularly true with fibers, like jute, rich in lignin. 45 With such fibers production of a full white or complete bleaching is attended with too much loss in weight or too much "tendering"; that is weakening of the fiber.

I have found that much better results can 50 be obtained by a special method of bleaching whereby it is possible to obtain an equal degree of bleaching with considerably less bleaching agent or, in using the same amount of bleaching agent a much greater bleaching 55 result can be attained, and with the fur-

ther unexpected result of a lessening in the usual loss of weight and tendering, thereby making it possible to secure a full bleach in some fibers, like jute, usually regarded as too refractory for a white bleach. Furthermore in this special method several other results are accomplished which do not follow from the use of the ordinary methods; these results being a diminution in the total ash of the fiber and a diminution in the amount 60 of ether extract—the latter representing fats, resins, etc. Why these results should follow I cannot say and content myself with noting the results without speculation as to the reason. Sometimes the reduction in ash 65 and ether content by the new method is astonishingly great. In one particular case a jute with about 14 per cent total ash, bleached by the ordinary methods still carried 10 per cent ash while when treated by 70 the present method and completely bleached it carried but two per cent.

From the facts, it appears that although ordinary bleaching agents (chlorin and bleaching liquor) are used in my method and 75 an unusually effective bleach is secured, the agents are doing something more than bleaching and since the extra effects are particularly noteworthy with fibers rich in lignin, that the extra effects are due to reaction with non-cellulosic components of the fiber other than lignin. Whatever the reason 80 the facts are as stated.

In the present invention, the fiber is first 85 treated with a small amount of bleaching 90 solution, this bleaching solution being made from bleaching powder in the ordinary way or in any other way as by leading chlorin into a solution of alkali. The liquor is, as is 95 usual with bleaching liquors, slightly alkaline. The amount used on the fiber is usually around 10 per cent of the total amount of 100 bleaching liquor which would be required to effect a substantial commercial bleaching action; in other words the amount here used 105 is, from the bleaching standpoint, extremely small. As soon as the bleaching liquor is incorporated into the pulp I treat at once with gaseous chlorin; blowing it into the 110 pulp or otherwise contacting it with the fiber to be treated. In working with pulped fiber I ordinarily take a 3 to 5 per cent pulp, stir the required amount of bleaching liquor into this and then blow chlorin into the pulp for the time necessary to effect the

action desired—say about 10 to 15 minutes with a slow introduction of chlorin. In operating in this way, the material is attacked practically simultaneously by an 5 alkaline bleaching liquor and by a solution of chlorin; this solution being, in large part, of chlorin as such. Chlorin on contact with water does not hydrolyze into hypochlorous and hydrochloric acids at once but remains 10 for a time as a solution of chlorin itself. And when hydrolysis occurs, it goes to a balance or a dynamic equilibrium between unhydrolyzed chlorin and its hydrolyzed reaction products, hypochlorous and hydro- 15 chloric acids. In the presence of hypochlorite (added as bleaching liquor) this hydrolysis is correspondingly retarded. The net result in the present process is that for a time the fiber is exposed both to the action 20 of a hypochlorite, hypochlorous acid, and to that of chlorin itself; something which seems to be necessary in accomplishing the present results. In these actions which I am now discussing while bleaching occurs, the non- 25 fibrous constituents, etc., which encrust the fibers are attacked and either oxidized or rendered water soluble or alkali soluble. After the requisite amount of chlorin has been introduced, this amount being usually 30 equal to about 50 per cent of the total bleaching agent required, the fiber is washed, in certain cases, the slight amount of hydrochloric acid present is neutralized with caustic soda or lime, and the fiber is finally put 35 through the usual bleach with bleaching liquor; the amount of bleach used being diminished however to allow for the bleaching agent used in the two prior stages. For an equal degree of bleaching, the total amount 40 of bleaching agent used in the three bleaching steps of the present process is considerably less than by either of the older methods hereinbefore described; or, for an equal amount of bleaching agent considerably 45 more bleaching is effected. And in some cases, and particularly with ligniferous fibers, as with the jute mentioned, with kraft pulp, etc., bleaching results can be accomplished which are impossible by any of the 50 known methods; that is without undue loss of weight and tendering.

Most vegetable fibers contain cellulose and in addition the bodies which collectively are known as lignin; the proportion of lignin 55 and cellulose varying from fiber to fiber. Some fibers, like cotton, contain very little

lignin while others, like jute, are rich in lignin and relatively poor in cellulose. Lignin is considerably more reactive chemically than is cellulose; a fact which is responsible both for the loss of weight and the tendering occurring in any drastic bleaching of fibers rich in lignin. Chlorin attacks lignin forming products soluble in alkaline solution and the lignin is moreover susceptible to oxidation. In the usual methods, using chlorin any attempt to secure far-going bleaching of jute results in a great loss of fiber, in tendering, etc. But on the other hand although chlorin is used in the present 60 method the loss of fiber with fibers rich in lignin is not greater than in usual methods of treating fibers poor in lignin such as cotton, sulfite pulp and the like and the bleaching action is sufficient while there is 65 no tendering or weakening of the fiber. Bleaching liquor and chlorin acting together in very dilute solution, as is the case in my method of bleaching, for some reason do not exercise the deleterious effects of either as is 70 the case at the higher bleaching concentrations usually employed. The activity of this combination of reagents is great but it specifically attacks the coloring matter and encrustants which are relatively more susceptible to their action rather than the cellulose or the fiber structure. For this reason 75 the bleaching action is more effective than when either is used separately at the higher concentrations usually employed. 80

What I claim is:—

1. In bleaching fiber the process which comprises treating the fiber with bleaching liquor and with chlorin, followed by another treatment with bleaching liquor. 95

2. In bleaching fiber the process which comprises treating fiber simultaneously with bleaching liquor and with chlorin and subsequently treating with bleaching liquor.

3. In bleaching fiber the process which 100 comprises treating the fiber with bleaching liquor and with chlorin, washing and following by another treatment with bleaching liquor.

4. In bleaching fiber the process which 105 comprises treating fiber simultaneously with bleaching liquor and with chlorin, washing with an alkaline wash and subsequently treating with bleaching liquor.

In testimony whereof, I have hereunto 110 affixed my signature.

JOHN R. MACMILLAN.